

## UNITED STATES PATENT OFFICE.

EDWARD J. HOFFMAN, OF CHICAGO, ILLINOIS, ASSIGNOR TO NATIONAL COMPRESSED COAL COMPANY, OF WILMINGTON, DELAWARE, A CORPORATION OF DELAWARE.

## BINDER FOR BRIQUETS.

SPECIFICATION forming part of Letters Patent No. 759,443, dated May 10, 1904.

Application filed March 9, 1904. Serial No. 197,389. (No specimens.)

*To all whom it may concern:*

Be it known that I, EDWARD J. HOFFMAN, a citizen of the United States, residing at Chicago, in the county of Cook and State of Illinois, have invented certain new and useful Improvements in Binders for Briquets; and I do hereby declare that the following is a full, clear, and exact description thereof.

This invention relates to a novel binding composition or compound for use in making briquets of coal or lignite dust and also to the novel fuel briquet made by the use of such binding compound.

The object of the invention is to produce briquets which will not melt down under the action of the heat of the fire in burning and will at the same time resist the action of water when exposed to the action of the elements, so that they may be kept indefinitely without deterioration.

The invention consists in the matters hereinafter described, and pointed out in the appended claims.

A binding compound for briquets made in accordance with my invention consists of crude petroleum, rosin, soda-ash, and lime.

I have successfully carried out my invention by the use of the above-named ingredients in the following proportions: crude petroleum, sixty-six per cent.; rosin, eleven per cent.; soda-ash, eleven per cent.; lime, eleven per cent.

The above-named ingredients used in the proportions specified produce a binding material which when mixed with pulverized coal or lignite afford briquets having the characteristics of being hard and durable, non-fusible, insoluble in water, and therefore weatherproof, highly inflammable, and possessing great heat-producing capacity.

In addition to the ingredients specified I also purpose using in the compound oil of myrbane in the proportion of one per cent. This is used to deodorize the crude petroleum and avoid the presence in the place in which the fuel briquets are stored of any objectionable petroleum odor.

In making fuel briquets according to my

invention I proceed as follows: First, I mix the crude petroleum and oil myrbane and allow the mixture to stand for twenty-four hours, when the petroleum will have been deodorized. The crude oil, rosin, and soda-ash are then placed in a tank or vat, to which heat is applied by means of a steam-jacket or by direct heat of a fire. These materials are heated until fused, and the lime in a slaked condition (calcium hydrate) is then added. The heated mixture is thoroughly stirred, the resulting compound being semiliquid or having such consistency as to have some degree of fluidity. The semiliquid binding compound is then mixed with coal or lignite dust in the proportion of nine per cent. (9%) of the binding compound to ninety-one per cent. (91%) of the coal or lignite dust. The plastic mass formed by the admixture of the binding compound with the coal or lignite dust is then compressed or molded under pressure into briquets or "eglettes" of size suitable for use as fuel.

Efforts have heretofore been made both in this country and abroad to produce an entirely satisfactory binding compound for fuel briquets; but all such efforts have failed, either because the briquets became disintegrated when subjected to the heat of the fire or because they were unable to withstand the action of the elements and dissolved when exposed to moisture and changes of temperature.

I have found that the binding compound made as described possesses the advantage that it will not soften or melt when the briquet is subjected to heat, this result arising from the action of the soda-ash upon the rosin and crude petroleum, which acts with the latter ingredients and produce a compound which will burn without becoming softened or melting down when ignited. The compound described also resists the action of water or moisture, the lime added to the saponified compound serving to render the same insoluble in water. In other words, the soda-ash and lime form with the rosin and crude petroleum an insoluble compound. The fuel

briquets produced by the use of said binding compound therefore have the advantage of being unaffected by the weather and may be kept in storage indefinitely without change and without losing their heating capacity.

The fuel briquets made as described burn freely and give out great heat during the progress of combustion, the binding compound affording a largely-increased proportion of combustible matter in the briquets, and therefore enhancing the heat-producing capacity of the fuel. The soda-ash and lime added to the compound to prevent the melting down of the briquets under heat or their dissolution under the effect of moisture do not serve to retard combustion; but I find in burning the briquets that combustion is very complete and that the entire mass of each briquet is reduced to ashes.

I am aware that the use has been suggested heretofore of compounds to be burned as a fuel or to be mixed with pulverized coal, lignite, or the like to increase the heating capacity of the fuel embracing petroleum and rosin with lime as a saponifying agent or petroleum and rosin with soda as a saponifying agent. My binder differs from such prior compounds from the fact that it includes soda as the principal saponifying agent and lime, which is added to make the compound and the briquets made therefrom insoluble in water, and therefore weatherproof. I have found that lime if used alone would not only be ineffectual as a saponifying agent, because of its low or slight saponifying action, but to produce an approach to the necessary degree of saponification of the petroleum and rosin it would be necessary to use it in such large quantity as to give much too large a proportion of non-combustible matter in the compound. Moreover, if lime be used in too large a proportion it produces an injurious effect on the compound, it having been found that when lime is present in large quantity the lime through its chemical action produces such changes in the petroleum and rosin that the compound will soon lose largely its adhesive or binding effect. I therefore employ soda as the principal saponifying agent and lime in such proportion only as is necessary to make the compound insoluble in water. I have also found that a compound in which soda is used as a

saponifying agent without lime the compound is readily soluble in water and if briquets made therefrom be exposed to the weather or 55 to moisture they will soon disintegrate and fall apart.

I do not wish to be limited to the use of the exact ingredients hereinbefore named or to a compound in which the ingredients are used 60 in exactly the proportions specified, the main feature of my invention being a binding compound which includes crude petroleum, rosin, or a resinous material, soda-ash or equivalent alkali or chemical having the property of 65 saponifying or solidifying the crude petroleum, and rosin and lime or equivalent material adapted to make the saponified mass insoluble in water.

The use of oil of myrbane to deodorize the 70 petroleum is of great advantage, because doing away with the objectionable smell of petroleum which is liable to prevail in a storage-room or the house in which the fuel is used when the crude petroleum in the briquets is 75 not deodorized.

I claim as my invention—

1. A binding compound for fuel briquets, consisting of crude petroleum, rosin, soda-ash and lime. 80

2. A binding compound for fuel briquets, consisting of crude petroleum, rosin, soda-ash, lime and oil of myrbane.

3. A fuel briquet, consisting of coal or lignite dust, crude petroleum, rosin, soda-ash 85 and lime.

4. A fuel briquet consisting of coal or lignite dust, crude petroleum, rosin, soda-ash, lime and oil of myrbane.

5. The process of making a binding compound for fuel briquets, consisting of the steps of mixing oil of myrbane with crude petroleum to deodorize the latter, mixing the deodorized crude petroleum with rosin and soda-ash and adding lime to the mixture. 90

In testimony that I claim the foregoing as my invention I affix my signature, in presence of two witnesses, this 7th day of March, A. D. 1904.

EDWARD J. HOFFMAN.

Witnesses:

C. CLARENCE POOLE,  
GERTRUDE BRYCE.